# EUROPEAN PATENT SPECIFICATION

(11) **EP 0 162 890 B1**
(45) Date of publication and mention of the grant of the patent: **23.08.1989**
(21) Application number: 84904244.5
(22) Date of filing: 30.10.1984
(51) Int. Cl.: C10L 1/22, C10M 133/08, C10M 149/16, C07C 93/04

(54) **DEPOSIT CONTROL ADDITIVES - HYDROXY POLYETHER POLYAMINES**
HYDROXY-POLYÄTHERPOLYAMINE ALS ADDITIVE ZUR STEUERUNG DES NIEDERSCHLAGS
ADDITIFS DE REGULATION DE DEPOT - POLYAMINES DE POLYETHER HYDROXY

(30) Priority: 31.10.1983 US 547558; 31.10.1983 US 547559
(43) Date of publication of application: 04.12.1985
(73) Proprietor: CHEVRON RESEARCH AND TECHNOLOGY COMPANY, San Francisco, CA 94120 (US)
(72) Inventor: CAMPBELL, Curtis, B., Rodeo, CA 94572 (US)
(74) Representative: Kosmin, Gerald Emmanuel
(86) International application number: US8401759
(87) International publication number: WO8501956

(56) References cited:
- US-A- 3 030 197
- US-A- 3 231 619
- US-A- 4 247 301
- US-A- 4 251 670

## Description

### Field of the invention

This invention is directed to hydroxy polyether polyamines, to fuel compositions and lubricating oil compositions containing these compounds and to their use as either fuel additives or detergent or dispersancy additives in lubricating oils.

Numerous deposit-forming substances are inherent in hydrocarbon fuels. These substances when used in internal combustion engines tend to form deposits on and around constricted areas of the engine contacted by the fuel. Typical areas commonly and sometimes seriously burdened by the formation of deposits include carburettor ports, the throttle body and venturies, engine intake valves, etc.

Deposits adversely affect the operation of the vehicle. For example, deposits on the carburettor throttle body and venturies increase the fuel to air ratio of the gas mixture to the combustion chamber thereby increasing the amount of unburned hydrocarbon and carbon monoxide discharged from the chamber. The high fuel-air ratio also reduces the gas mileage obtainable from the vehicle.

Deposits on the engine intake valves when they get sufficiently heavy, on the other hand, restrict the gas mixture flow into the combustion chamber. This restriction, starves the engine of air and fuel and results in a loss of power. Deposits on the valves also increase the probability of valve failure due to burning and improper valve seating. In addition, these deposits may break off and enter the combustion chamber possibly resulting in mechanical damage to the piston, piston rings, engine head, etc.

The formation of these deposits can be inhibited as well as removed by incorporating an active detergent into the fuel. These detergents function to cleanse these deposit-prone areas of the harmful deposits, thereby enhancing engine performance and longevity. There are numerous detergent-type gasoline additives currently available which, to varying degrees, perform these functions.

Two complicating factors have, however, recently arisen. First, with the advent of automobile engines that require the use of nonleaded gasolines (to prevent disablement of catalytic converters used to reduce emissions), it has been found difficult to provide gasoline of high enough octane to prevent knocking and the concomitant damage which it causes. The chief problem lies in the area of the degree of octane requirement increase, herein called "ORI", which is caused by deposits formed by the commercial gasoline.

The basis of the ORI problem is as follows: each engine, when new, requires a certain minimum octane fuel in order to operate satisfactorily without pinging and/or knocking. As the engine is operated on any gasoline, this minimum octane increases and, in most cases, if the engine is operated in the same fuel for a prolonged period, will reach an equilibrium. This is apparently caused by an amount of deposits in the combustion chamber. Equilibrium is typically reached after 5000 to 15000 miles of automobile operation.

The octane requirement increase in particular engines used with commercial gasolines will vary at equilibrium from 5 or 6 octane units to as high as 12 or 15 units, depending upon the gasoline compositions, engine design and type of operation. The seriousness of the problem is thus apparent. A typical automobile with a research octane requirement of 85, when new, may after a few months of operation require 97 research octane gasoline for proper operation, and little unleaded gasoline of that octane is available. The ORI problem also exists in some degree with engines operated on leaded fuels. U.S. Patent Nos. 3,144,311; 3,146,203; and 4,247,301 disclose lead-containing fuel compositions having reduced ORI properties.

The ORI problem is compounded by the fact that the most common method for increasing the octane rating of unleaded gasoline is to increase its aromatic content. This, however, eventually causes an even greater increase in the octane requirement. Moreover, some of presently used nitrogen-containing compounds used as deposit-control additives and their mineral oil or polymer carriers may also significantly contribute to ORI in engines using unleaded fuels.

It is, therefore, particularly desirable to provide deposit control additives which effectively control the deposits in intake systems of engines, without themselves eventually contributing to the problem.

The second complicating factor relates to oil solubility of the fuel additives. Fuel additives, due to their higher boiling point over gasoline itself, tend to accumulate on surfaces in the combustion chamber. This accumulation of the additive eventually finds its way into the lubricating oil via a "blow-by" process. In some cases this process may be of no concern as the fuel additives will be inert and compatible in the oil. However, if the additive is incompatible in the lubricating oil a serious problem develops as the accumulation of the additive results in an emulsion-like sludge which is detrimental to efficient operation. Therefore, it is particularly desirable that the gasoline additive be oil compatible.

The present invention also relates to lubricating oil compositions containing hydroxy polyether polyamines which contribute dispersancy and detergency to the compositions.

Lubricating oil compositions, particularly for use in internal combustion engines, have long performed many functions other than simply lubricating moving parts. Modern-day, highly compounded lubricating oil compositions provide anti-wear, anti-oxidant, extreme-pressure and anti-rust protection in addition to maintaining the cleanliness of the engine by detergency and dispersancy. Many lubricating oil additives are well known for accomplishing these functions. For maintaining engine cleanliness, a well-known class of ashless detergents which have been found to be particularly useful are polyoxyalkylene carbamates.

Polyether amine-type fuel additives for deposit control and lubricating oil dispersancy are well-known but have traditionally been surfactant-type molecules having a large, non-polar hydrophobic end or "tail", for instance, a hydrocarbyl capped polyether moiety, and a polar, hydrophilic amine or polyamine end. Examples of these type of compositions may be found in U.S. Patent No. 4,247,301; U.S. Patent No. 4,160,648; and EP-A-0100665. In U.S. Patent No. 3030197 there are disclosed thermally stable distillate fuels which have been stabilized by means of an additive which is an oxyalkylation product formed by reacting certain polyamines with certain epoxides in an excess amount so that all the nitrogen atoms of the polyamine reactant will be attached to an oxyalkylene group derived from the epoxide reactant.

In the present invention, however, a composition has been discovered which in gasoline fuel functions as a deposit control additive and in lubricating oil functions as a dispersant and detergent additive which has a single hydroxyl group in the non-polar hydrophobic portion of the molecule. These additives contain block co-polymer polyethers in which there is no hydrocarbyl cap. Moreover, this additive is compatible in the lubricating oil.

In accordance with the invention, additives are provided which, when added to fuels or used as fuel concentrates, are effective in cleaning and maintaining the cleanliness of engine intake systems and when added at from 0.01 to 10 weight percent to lubricating oil, are effective in providing dispersancy and detergency to the oil. The additives consist of certain fuel and lubricating oil soluble hydroxy polyoxyalkylene amines or polyamines. These additives have the following general formula: wherein:
R' and R" independently=H, or alkyl groups of 1 to 4 carbon atoms, and at least one of R' and R" has at least 2 carbon atoms;
R"' and R^{lv} independently=H or CH₃;
R" and R" independently=H or where
z=1 to 5; and
x and y independently are integers from 1 to 30.

The compositions may be either mono or polyamines, but polyamines are preferred. The additive compounds have molecular weights in the range from 500 to 2000, preferably from 700 to 1200.

The invention is based on our finding that the hydrophobic portion of a polyether polyamine fuel additive may contain an "uncapped" hydroxyl group, provided that the polyether is a co-polymer and that the portion of the co-polymer having the hydroxyl group has more carbon atoms per unit than the other portion of the block co-polymer. Thus, a preferred compound is composed of a block co-polymer in which the hydroxyl-containing portion is composed of poly(butylene glycol) and the other portion is composed of poly(ethylene glycol). Furthermore, it is preferred that R' has at least 2 carbon atoms, and R", R'" and R'" are H.

As fuel additives, the compositions are selected to provide solubility in fuel compositions and deposit control activity without contributing to octane requirement increase (ORI).

In the fuel composition, the desired concentration of the additive will vary according to fuel type and quality and the presence or absence of other additives, etc. Generally, however, the concentration will be from 250 parts per million (ppm) by weight to 5000 ppm by weight. The preferred concentration is from 300 ppm to 2000 ppm.

It is also contemplated that the additive compositions may be used as concentrates, and could be used as additives to fuels subsequent to their preparation. In concentrates, the weight percent of these additives will usually range from 0.3 to 50 weight percent. The concentrate would ordinarily comprise an inert stable oleophilic organic solvent and the carrier of said solvent boiling in the range of from 150° to 400°F (65.5 to 204.4°C) and the concentrate would preferably contain from about 10 to 50 weight percent of the additive compound.

As lubricating oil additives, the specific compositions are selected to provide solubility in lubricating oil compositions with dispersant activity, without contributing to deposit formation in the lubricating oil composition. In general, the addition to the oil of from 0.01 to 10 weight percent of an additive of this invention is effective in providing dispersancy and detergency to the oil.

The oils which find use in this invention are oils of lubricating viscosity derived from petroleum or synthetic sources. Oils of lubricating viscosity normally have viscosities in the range of 35 to 50,000 Saybolt Universal Seconds (SUS) at 37.6°C and more usually from about 50 to 10,000 SUS at 37.6°C. Examples of such base oils are naphthenic bases, paraffin base and mixed base mineral oils, synthetic oils; for example, alkylene polymers, such as the polymers of propylene, butylene, etc., and mixtures thereof.

Usually included in the oils besides the subject additives are such additives as dispersant/detergents, rust inhibitors, antioxidants, oiliness agents, foam inhibitors, viscosity index improvers, pour point depressants, etc. Usually, these other additives will be present in amounts of from about 0.5 to 15 weight percent of the total composition. Generally, each of the additives will be present in the range from about 0.01 to 5 weight percent of the total composition.

It is also contemplated that the additive compositions may be used as lubricating oil concentrates, and could be used as additive to lubricating oils subsequent to their preparation. In concentrates, the weight percent of these additives will usually range from about 10 to 90 weight percent.

The additive compounds can be prepared by a variety of known processes. In a preferred embodiment, an appropriate hydroxy-substituted amine, containing both the desired amino moiety and the appropriate hydroxy-terminated alkyl moiety, is first reacted to form an alkali alkoxide salt which is then reacted with an appropriate alkylene oxide or other oxylating agent. The resulting polyether amine is then reacted with a second epoxyalkane having the desired R' or R" brand alkyl groups, at least one of which has more than 2 carbon atoms. Upon termination of the second epoxidation, a block co-polymer is produced having a hydroxyl group near the end of the second polyether moiety.

In another embodiment, a halohydroxyalkylene, preferably chlorohydroxyalkylene is first reacted at the hydroxy terminus with an appropriate alkylene oxide. The halo group is then reacted with an amine or polyamine, preferably in excess to yield the hydroxy poly(oxyalkylene) amines or polyamines of this invention. Examples of suitable halohydroxyalkylenes include 2-chloroethanol, 2-chloropropanol, and the like.

The preparation of the compound is illustrated by, but not intended to be limited to, the following example for the preparation of Example

A solution of 10 ml (139 mmols) 2 - (2 - aminoethoxy)ethanol in 275 ml of dioxane was azeotropically dried by distilling off 25 ml in a nitrogen atmosphere. The solution was cooled to 0° to 5°C in an ice bath and approx. 6.5 gms (approx. 167 mmols) of potassium metal cut into small pieces was added with stirring while flushing the flask with nitrogen. After the addition was completed, the slurry was warmed to room temperature over 48 hours, and any unreacted-potassium metal (approx. 1 gm, 26 mmols) was removed from the reaction.

The resulting slurry was heated to approx. 90°C and 100 ml (1.16 moles) of distilled 1,2-epoxybutane was added over 30 minutes. After this addition, the reaction was stirred with heating for 30 minutes and then cooled to room temperature and stirred for 16 hours.

The reaction was quenched by adding approx. 200 ml of t-butanol and stirring 30 minutes, followed by approx. 50 ml of water. The reaction was diluted with 300 ml ether and extracted with two 100 ml portions of water.

Sufficient 10% aqueous HCI was added to the water extraction to bring the aqueous layer to about pH 7.

The product was washed with additional water, and the organic layer dried over anhydrous K_{Z}C0₃. After filtration and concentration in vacuo, 98.2 gms (94% mass recovery) of a yellow oil was isolated: Basic N=₀._{84%}; MW=759±2; hydroxyl number=125; and C=65.76%, H=11.31%, N=0.85%.

By Carbon ¹³ NMR, no secondary amine was present indicating no polymerization at the amine nitrogen took place.

To test for deposit control activity, the hydroxy polyether amines prepared above were blended in gasoline to various concentrations and were run in the ASTM/CFR Single-Cylinder Engine Test.

In carrying out the tests, a Waukesha CFR single-cylinder engine is used. The run is carried out for 15 hours, at the end of which time the intake valve is removed, washed with hexane and weighed. The previously determined weight of the clean valve is subtracted from the weight of the valve. The difference between the two weights is the weight of the deposit with a lesser amount of deposit measured connoting a superior additive. The operating conditions of the test are as follows: water jacket temperature 100°C; manifold vacuum of 29.5 cm Hg, intake mixture temperature of 50.2°C; air-fuel ratio of 12; ignition spark timing of 40° BTC; engine speed is 1800 rpm; and the crankcase oil is a commercial 30 W oil. The amount of carbonaceous deposit in milligrams on the intake valves is measured and reported in the following Table I.

All specific embodiments of the invention have been described in detail. It should be understood that the invention is to be given the broadest possible interpretation within the terms of the following claims.

## Claims

1. A fuel- and lubricating oil-soluble additive for engine deposit control, said additive being a hydroxy polyether amine or polyamine in which the polyether moiety is a copolymer, that portion of the copolymer having the hydroxy group containing more carbon atoms per unit than the other portion of the copolymer, wherein the additive is represented by the general formula: wherein: .
R' and R" independently are hydrogen or alkyl groups having from 1 to 4 carbon atoms, at least one of R' and R" having at least 2 carbon atoms;
R"' and R^{iv} independently are hydrogen or methyl;
R" and R"' independently are hydrogen or where
z is an integer from 1 to 5; and
x and y independently are integers from 1 to 30, and wherein said additive has a molecular weight in the range from 500 to 2000.

2. An additive as claimed in Claim 1, wherein said molecular weight is in the range from 700 to 1200.

3. An additive as claimed in Claim 1 or 2, wherein R' is ethyl, R" is hydrogen, R"' and R'" are hydrogen, R" and R^{vi} are hydrogen, x has an average value of 9 and y is 2.

4. A fuel composition comprising a major proportion of a hydrocarbon fuel boiling in the gasoline range, and a minor proportion of an additive as claimed in any one of Claims 1 to 3.

5. A fuel composition as claimed in Claim 4, wherein the concentration of said additive in said fuel is from 250 parts per million to 5000 parts per million by weight.

6. A fuel composition as claimed in Claim 5, wherein said concentration is from 300 ppm by weight to 2000 ppm by weight.

7. A concentrate comprising an inert stable oleophilic organic solvent boiling in the range from 65.5° to 204.4°C and from 0.3 to 50 weight percent of an additive as claimed in any of Claims 1 to 3.

8. A lubricating oil composition comprising a major proportion of an oil of lubricating viscosity, and a minor proportion of an additive as claimed in any one of Claims 1 to 3.

9. A lubricating oil composition as claimed in Claim 8, wherein said minor proportion of the additive comprises from 0.01 to 10 weight percent of the total composition.

## Patentansprüche

1. Treibstoff- und schmieröllösliches Additiv für eine Bekämpfung von Ablagerungen in Motoren, wobei dieses Additiv ein Hydroxypolyetheramin oder -polyamin ist, in welchem der Polyetheranteil ein Copolymeres ist und der Teil des Copolymeren mit der Hydroxygruppe mehr Kohlenstoffatome pro Einheit enthält als der andere Teil des Copolymeren, und wobei das Additiv durch die allgemeine Formel wiedergegeben wird, worin R' und R" unabhängig voneinander Wasserstoff oder Alkylgruppen mit 1 bis 4 Kohlenstoffatomen sind, wenigstens einer der Substituenten
R' und R" wenigstens zwei Kohlenstoffatome aufweist,
R"' und R'" unabhängig voneinander Wasserstoff oder Methyl sind, R" und R^{vi} unabhängig voneinander Wasserstoff oder sind, wobei
z eine ganze Zahl von 1 bis 5 ist, und
x und y unabhängig voneinander ganze Zahlen von 1 bis 30 sind, und wobei das Additiv ein Molekulargewicht im Bereich von 500 bis 2000 besitzt.

2. Additiv nach Anspruch 1, wobei das Molekulargewicht im Bereich von 700 bis 1200 liegt.

3. Additiv nach Anspruch 1, wobei R' Ethyl ist, R" Wasserstoff ist, R"' und R'" Wasserstoff sind, R" und R^{vi} Wasserstoff sind und x einen durchschnittlichen Wert von 9 besitzt und y 2 ist.

4. Treibstoffzubereitung aus einer größeren Menge eines Kohlenwasserstofftreibstoffs, der im Benzinbereich siedet, und einem kleineren Teil eines Additivs gemäß einem der Ansprüche 1 bis 3.

5. Triebstoffzusammensetzung nach Anspruch 4, wobei die Konzentration des Additivs in dem Treibstoff 250 Teile pro Million bis 5000 Teile pro Million, bezogen auf das Gewicht, beträgt.

6. Treibstoffzusammensetzung nach Anspruch 5, wobei diese Konzentration 300 ppm, bezogen auf das Gewicht, bis 2000 ppm, bezogen auf das Gewicht, beträgt.

7. Konzentrat aus einem inerten stabilen oleophilen organischen Lösungsmittel, das im Bereich von 65,5° bis 204,4°C siedet, und 0,3 bis 50 Gew.-% eines Additivs gemäß einem der Ansprüche 1 bis 3.

8. Schmierölzubreitung aus einer größeren Menge eines Öls mit Schmierviskosität und einer kleineren Menge eines Additivs gemäß einem der Ansprüche 1 bis 3.

9. Schmierölzubreitung nach Anspruch 8, wobei der kleinere Anteil des Additivs 0,01 bis 10 Gew.-% der gesamten Zubereitung ausmacht.

## Revendications

1. Additif soluble dans les carburants et les huiles lubrifiantes, destiné à limiter le dépôt dans les moteurs, ledit additif étant une hydroxypolyéther-amine ou -polyamine dans laquelle le groupement polyéther est un cdpolymère, la portion du copolymère portant le groupe hydroxy contenant un nombre d'atomes de carbone par motif supérieur à celui de l'autre portion du copolymère, l'additif répondant à la formule générale: dans laquelle:
R' et R" représentent indépendamment l'hydrogène ou des groupes alkyle ayant 1 à 4 atomes de carbone, au moins l'un des groupes R' et R" ayant au moins 2 atomes de carbone;
R"' et R'" représentent indépendamment l'hydrogène ou un groupe méthyle;
R" et R"' représentent indépendamment l'hydrogène ou un groupe dans lequel
z est un nombre entier de 1 à 5; et
x et y représentent indépendamment des nombres entiers de 1 à 30,
ledit additif ayant un poids moléculaire de 500 à 2000.

2. Additif suivant la revendication 1, dans lequel le poids moléculaire est compris dans l'intervalle de 700 à 1200.

3. Additif suivant la revendication 1 ou 2, dans lequel R' représente un groupe éthyle, R" représente l'hydrogène, R'" et R'" représentent l'hydrogène, R" et R"' représentent l'hydrogène, x possède une valeur moyenne de 9 et y est égal à 2.

4. Composition de carburant comprenant une forte proportion d'un carburant hydrocarboné bouillant dans la plage de l'essence et une faible proportion d'un additif suivant l'une quelconque des revendications 1 à 3.

5. Composition de carburant suivant la revendication 4, dans laquelle la concentration de l'additif dans ledit carburant est comprise dans l'intervalle de 250 parties par million à 5000 parties par million, en poids.

6. Composition de carburant suivant la revendication 5, dans laquelle la concentration va de 300 ppm, en poids, à 2000 ppm, en poids.

7. Concentré comprenant un solvant organique stable oléophile inerte, stable, bouillant dans la plage de 65,5° à 204,4°C et 0,3 à 50% en poids d'un additif suivant l'une quelconque des revendications 1 à 3.

8. Composition d'huile lubrifiante contenant une forte proportion d'une huile de viscosité propre à la lubrification et une faible proportion d'un additif suivant l'une quelconque des revendications 1 à 3.

9. Composition d'huile lubrifiante suivant la revendication 8, dans laquelle la faible proportion de l'additif représente 0,01 à 10% en poids de la composition totale.
